



US005168094A

# United States Patent [19]

Shuttleworth et al.

[11] Patent Number: 5,168,094

[45] Date of Patent: \* Dec. 1, 1992

[54] MIXTURE OF YELLOW AND CYAN DYES  
TO FORM GREEN HUE FOR COLOR  
FILTER ARRAY ELEMENT

[75] Inventors: Leslie Shuttleworth; Helmut Weber,  
both of Webster, N.Y.

[73] Assignee: Eastman Kodak Company,  
Rochester, N.Y.

[\*] Notice: The portion of the term of this patent  
subsequent to Dec. 4, 2007 has been  
disclaimed.

[21] Appl. No.: 693,500

[22] Filed: Apr. 30, 1991

[51] Int. Cl.<sup>5</sup> B41M 5/035; B41M 5/38

[52] U.S. Cl. 503/227; 428/195;  
428/210; 428/412; 428/913; 428/914; 430/7;  
430/200; 430/201; 430/945; 359/885

[58] Field of Search 8/471; 156/235, 271;  
350/311; 428/195, 209, 480, 913, 914, 210;  
430/7, 200, 201, 945; 503/227

## [56] References Cited

### U.S. PATENT DOCUMENTS

4,952,553 8/1990 Kanto et al. 503/227  
4,975,410 12/1990 Weber et al. 503/227

### FOREIGN PATENT DOCUMENTS

279467 8/1988 European Pat. Off. 503/227  
327063 8/1989 European Pat. Off. 503/227

Primary Examiner—Bruce H. Hess  
Attorney, Agent, or Firm—Harold E. Cole

### [57] ABSTRACT

A thermally-transferred color filter array element comprising a support having thereon a polymeric dye image-receiving layer containing a thermally-transferred image comprising a repeating pattern of colorants, one of the colorants being a mixture of a yellow dye and a cyan dye to form a green hue, said cyan dye having the formula:



20 Claims, No Drawings

**MIXTURE OF YELLOW AND CYAN DYES TO  
FORM GREEN HUE FOR COLOR FILTER ARRAY  
ELEMENT**

This invention relates to the use of a mixture of a yellow dye and a cyan dye to form a green hue for a thermally-transferred color filter array element which is used in various applications such as a liquid crystal display device.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Pat. No. 4,621,271 by Brownstein entitled "Apparatus and Method For Controlling A Thermal Printer Apparatus," issued Nov. 4, 1986, the disclosure of which is hereby incorporated by reference.

Another way to thermally obtain a print using the electronic signals described above is to use a laser instead of a thermal printing head. In such a system, the donor sheet includes a material which strongly absorbs at the wavelength of the laser. When the donor is irradiated, this absorbing material converts light energy to thermal energy and transfers the heat to the dye in the immediate vicinity, thereby heating the dye to its vaporization temperature for transfer to the receiver. The absorbing material may be present in a layer beneath the dye and/or it may be admixed with the dye. The laser beam is modulated by electronic signals which are representative of the shape and color of the original image, so that each dye is heated to cause volatilization only in those areas in which its presence is required on the receiver to reconstruct the color of the original object. Further details of this process are found in GB 2,083,726A, the disclosure of which is hereby incorporated by reference.

Liquid crystal display devices are known for digital display in electronic calculators, clocks, household appliances, audio equipment, etc. Liquid crystal displays are being developed to replace cathode ray tube technology for display terminals. Liquid crystal displays occupy a smaller volume than cathode ray tube devices with the same screen area. In addition, liquid crystal display devices usually have lower power requirements than corresponding cathode ray tube devices.

There has been a need to incorporate a color display capability into such monochrome display devices, particularly in such applications as peripheral terminals using various kinds of equipment involving phototube

display, mounted electronic display, or TV-image display. Various attempts have been made to incorporate a color display using a color filter array element into these devices. However, none of the color array elements for liquid crystal display devices so far proposed have been successful in meeting all the users' needs.

One commercially-available type of color filter array element which has been used in liquid crystal display devices for color display capability is a transparent support having a gelatin layer thereon which contains dyes having the additive primary colors red, green and blue in a mosaic pattern obtained by using a photolithographic technique. To prepare such a color filter array element, a gelatin layer is sensitized, exposed to a mask for one of the colors of the mosaic pattern, developed to harden the gelatin in the exposed areas, and washed to remove the unexposed (uncrosslinked) gelatin, thus producing a pattern of gelatin which is then dyed with dye of the desired color. The element is then recoated and the above steps are repeated to obtain the other two colors. Misalignment or improper deposition of color materials may occur during any of these operations. This method therefore contains many labor-intensive steps, requires careful alignment, is time-consuming and very costly. Further details of this process are disclosed in U.S. Pat. No. 4,081,277. U.S. Pat. No. 4,786,148 also discloses a color filter array element which employs certain pigments.

Color liquid crystal display devices generally include two spaced glass panels which define a sealed cavity which is filled with a liquid crystal material. For actively-driven devices, a transparent electrode is formed on one of the glass panels, which electrode may be patterned or not, while individually addressable electrodes are formed on the other of the glass panels. Each of the individual electrodes has a surface area corresponding to the area of one picture element or pixel. If the device is to have color capability, a color filter array with, e.g., red, green and blue color areas must be aligned with each pixel. Depending upon the image to be displayed, one or more of the pixel electrodes is energized during display operation to allow full light, no light or partial light to be transmitted through the color filter areas associated with that pixel. The image perceived by a user is a blending of colors formed by the transmission of light through adjacent color filter areas.

In forming such a liquid crystal display device, the color filter array element to be used therein may have to undergo rather severe heating and treatment steps during manufacture. For example, a transparent conducting layer, such as indium tin oxide (ITO), is usually vacuum sputtered onto the color filter array element which is then cured and patterned by etching. The curing may take place at temperatures elevated as high as 200° C. for times which may be as long as one hour or more. This is followed by coating with a thin polymeric alignment layer for the liquid crystals, such as a polyimide, followed by another curing step for up to several hours at an elevated temperature. These treatment steps can be very harmful to many color filter array elements, especially those with a gelatin matrix.

It is thus apparent that dyes used in color filter arrays for liquid crystal displays must have a high degree of heat and light stability above the requirements desired for dyes used in conventional thermal dye transfer imaging.

While a green dye may be formed from a mixture of one or more cyan and one or more yellow dyes, not all

such combinations will produce a dye mixture with the correct hue for a color filter array. Further, when a dye mixture with the correct hue is found, it may not have the requisite stability to heat and light. An additional requirement is that no single dye of the mixture can have an adverse effect on the stability to heat and light or crystallinity of any of the other dye components.

EPA's 327,063 and 279,467 and U.S. Pat. No. 4,952,553 describe oxopyrroline dyes useful in thermal printing. There is no disclosure in these applications, however, that the dyes may be mixed with yellow dyes to form a green dye useful in a color filter array.

U.S. Pat. No. 4,975,410 describes the use of a mixture of a yellow dye and a cyan dye to form a green hue for a color filter array element. However, the cyan dyes employed in the patent are different from the cyan dyes employed herein.

It would be desirable to provide a color filter array element having high quality, good sharpness and which could be obtained easily and at a lower price than those of the prior art. It would also be desirable to provide such a color filter array element having a green dye of the correct hue and which would have good stability to heat and light.

These and other objects are achieved in accordance with this invention which comprises a thermally-transferred color filter array element comprising a support having thereon a polymeric dye image-receiving layer containing a thermally-transferred image comprising a repeating pattern of colorants, one of the colorants being a mixture of a yellow dye and a cyan dye to form a green hue, said cyan dye having the formula:



wherein:

R¹ represents hydrogen; a substituted or unsubstituted alkyl group having from 1 to about 8 carbon atoms such as methyl; ethyl, propyl, isopropyl, butyl, pentyl, hexyl, methoxyethyl, benzyl, 2-methane-, 2-hydroxyethyl, 2-cyanoethyl, methoxycarbonylmethyl, etc.; a cycloalkyl group having from about 5 to about 8 carbon atoms, such as cyclohexyl, cyclopentyl, etc.; or an alkenyl group having from about 2 to about 8 carbon atoms, such as —CH<sub>2</sub>CH=CH<sub>2</sub>, —CH<sub>2</sub>CH=CH—CH=CH<sub>2</sub>, —CH<sub>2</sub>CHCHBr, or —CH<sub>2</sub>CH=CHCH<sub>2</sub>OCH<sub>3</sub>;

R² and R³ each independently represents hydrogen; a substituted or unsubstituted alkyl group having from 1 to about 8 carbon atoms, such as those listed above for R¹; or a cycloalkyl group having from about 5 to about 8 carbon atoms, such as those listed above for R¹;

or R² and R³ may be taken together to form a ring such as pentamethylene, hexamethylene, etc.; or a 5- or 6-membered heterocyclic ring may be formed with R² or R³, the nitrogen to which R² or R³ is attached, and J which is an alkyl group ortho to the carbon attached to the nitrogen atom;

each J independently represents hydrogen; halogen, such as chlorine, bromine, or fluorine; a substituted or unsubstituted alkyl or alkoxy group (such as methoxy, ethoxy, methoxyethoxy 2-cyanoethoxy) having from 1 to about 6 carbon atoms; or two adjacent J's may represent the atoms necessary to form a 6-membered, fused, aromatic, carbocyclic ring; and n is from 1 to 4.

In a preferred embodiment of the invention, R¹ in the above formula is CH<sub>2</sub>CH=CH<sub>2</sub>, R² and R³ are each n-C<sub>4</sub>H<sub>9</sub> and J is hydrogen. In another preferred embodiment, a 6-membered heterocyclic ring is formed with R³, the nitrogen to which R³ is attached, and J which is ortho to the carbon attached to the nitrogen atom; and R² is n-C<sub>4</sub>H<sub>9</sub> or C<sub>2</sub>H<sub>5</sub>.

Specific cyan dyes useful in the invention include the following:



| Compound | R¹                                                                | R²                                                             | R³                                                                                          | J                                                   |
|----------|-------------------------------------------------------------------|----------------------------------------------------------------|---------------------------------------------------------------------------------------------|-----------------------------------------------------|
| 1        | CH <sub>2</sub> CH=CH <sub>2</sub>                                | n-C <sub>4</sub> H <sub>9</sub>                                | n-C <sub>4</sub> H <sub>9</sub>                                                             | H                                                   |
| 2        | C <sub>2</sub> H <sub>5</sub>                                     | n-C <sub>4</sub> H <sub>9</sub>                                | n-C <sub>4</sub> H <sub>9</sub>                                                             | H                                                   |
| 3        | H                                                                 | C <sub>2</sub> H <sub>5</sub>                                  | C <sub>2</sub> H <sub>4</sub> OC <sub>2</sub> H <sub>4</sub> OC <sub>2</sub> H <sub>5</sub> | H                                                   |
| 4        | CH <sub>2</sub> C <sub>6</sub> H <sub>5</sub>                     | n-C <sub>4</sub> H <sub>9</sub>                                | n-C <sub>4</sub> H <sub>9</sub>                                                             | H                                                   |
| 5        | CH <sub>2</sub> OCH <sub>3</sub>                                  |                                                                | CH <sub>2</sub> CH <sub>2</sub> OCH <sub>2</sub> CH <sub>2</sub>                            | 3-OCH <sub>3</sub>                                  |
| 6        | H                                                                 | C <sub>2</sub> H <sub>5</sub>                                  | C <sub>2</sub> H <sub>5</sub>                                                               | 3-OCH <sub>3</sub>                                  |
| 7        | CH <sub>3</sub>                                                   | H                                                              | C <sub>2</sub> H <sub>5</sub>                                                               | 2-OCH <sub>3</sub>                                  |
| 8        | CH <sub>2</sub> C <sub>6</sub> H <sub>4</sub> -p-OCH <sub>3</sub> |                                                                | (CH <sub>2</sub> ) <sub>4</sub>                                                             | 2,6-Cl                                              |
| 9        | s-C <sub>6</sub> H <sub>11</sub>                                  | CH <sub>2</sub> CH <sub>2</sub> OC <sub>2</sub> H <sub>5</sub> | CH <sub>2</sub> CH <sub>2</sub> OC <sub>2</sub> H <sub>5</sub>                              | 2-(C <sub>2</sub> H <sub>4</sub> OCH <sub>3</sub> ) |
| 10       | CH <sub>2</sub> C <sub>6</sub> H <sub>5</sub>                     | CH <sub>2</sub> CH=CH <sub>2</sub>                             | CH <sub>2</sub> CH=CH <sub>2</sub>                                                          | 3Br                                                 |

-continued



| DYE | R <sup>1</sup>                                | R <sup>2</sup>                   | J                 |
|-----|-----------------------------------------------|----------------------------------|-------------------|
| 14  | CH <sub>2</sub> CH=CH <sub>2</sub>            | n-C <sub>4</sub> H <sub>9</sub>  | H                 |
| 15  | CH <sub>2</sub> CH=CH <sub>2</sub>            | C <sub>2</sub> H <sub>5</sub>    | H                 |
| 16  | CH <sub>2</sub> CH=CH <sub>2</sub>            | H                                | H                 |
| 17  | H                                             | C <sub>2</sub> H <sub>5</sub>    | 7-CH <sub>3</sub> |
| 18  | CH <sub>2</sub> C <sub>6</sub> H <sub>5</sub> | C <sub>2</sub> H <sub>5</sub>    | 7-CH <sub>3</sub> |
| 19  | CH <sub>3</sub>                               | CH <sub>2</sub> OCH <sub>3</sub> | Cl                |

Any yellow dye may be employed in the invention to 50  
be mixed with the cyan dye described above. For example, there may be employed dicyanovinylaniline dyes as disclosed in U.S. Pat. Nos. 4,701,439 and 4,833,123 and JP 60/28,451, the disclosures of which are hereby incorporated by reference, e.g., 55



merocyanine dyes as disclosed in U.S. Pat. Nos. 65  
4,743,582 and 4,757,046, the disclosures of which are  
hereby incorporated by reference, e.g.,

pyrazolone arylidene dyes as disclosed in U.S. Pat. No. 4,866,029, the disclosure of which is hereby incorporated by reference; e.g.,



B

C

azophenol dyes as disclosed in JP 60/30,393, the disclosure of which is hereby incorporated by reference; e.g.,



azopyrazolone dyes as disclosed in JP 63/182,190 and JP 63/182,191, the disclosures of which are hereby incorporated by reference, e.g.,



pyrazolinedione arylidene dyes as disclosed in U.S. Pat. No. 4,853,366, the disclosure of which is hereby incorporated by reference, e.g.,



azopyridone dyes as disclosed in JP 63/39,380, the disclosure of which is hereby incorporated by reference, e.g.,



quinophthalone dyes as disclosed in EP 318,032, the disclosure of which is hereby incorporated by reference, e.g.,



azodiaminopyridine dyes as disclosed in EP 346,729, U.S. Pat. No. 4,914,077 and DE 3,820,313, the disclosures of which are hereby incorporated by reference, e.g.,



G azamethine dyes as disclosed in JP 01/176,591, EPA 279,467, JP 01/176,590, and JP 01/178,579, the disclosures of which are hereby incorporated by reference, e.g.,



H 55 nitrophenylazoaniline dyes as disclosed in JP 60/31,565, the disclosure of which is hereby incorporated by reference, e.g.,



I 65 pyrazolothiazole dyes as disclosed in U.S. Pat. No. 4,891,353, the disclosure of which is hereby incorporated by reference; arylidene dyes as disclosed in U.S. Pat. No. 4,891,354, the disclosure of which is hereby incorporated by reference; and dicyanovinylothiazole

dyes as disclosed in U.S. Pat. No. 4,760,049, the disclosure of which is hereby incorporated by reference.

As noted above, the dye image-receiving layer contains a thermally-transferred image comprising a repeating pattern of colorants in the polymeric dye image-receiving layer, preferably a mosaic pattern.

In a preferred embodiment of the invention, the mosaic pattern consists of a set of red, green and blue additive primaries.

In another preferred embodiment of the invention, each area of primary color and each set of primary colors are separated from each other by an opaque area, e.g., black grid lines. This has been found to give improved color reproduction and reduce flare in the displayed image.

The size of the mosaic set is not critical since it depends on the viewing distance. In general, the individual pixels of the set are from about 50 to about 600  $\mu\text{m}$  and do not have to be of the same size.

In a preferred embodiment of the invention, the repeating mosaic pattern of dye to form the color filter array element consists of uniform, square, linear repeating areas, with one color diagonal displacement as follows:



In another preferred embodiment, the above squares are approximately 100  $\mu\text{m}$ .

The color filter array elements prepared according to the invention can be used in image sensors or in various electro-optical devices such as electroscopic light valves or liquid crystal display devices. Such liquid crystal display devices are described, for example, in UK Patents 2,154,355; 2,130,781; 2,162,674 and 2,161,971.

Liquid crystal display devices are commonly made by placing a material, which is liquid crystalline at the operating temperature of the device, between two transparent electrodes, usually indium tin oxide coated on a substrate such as glass, and exciting the device by applying a voltage across the electrodes. Alignment layers are provided over the transparent electrode layers on both substrates and are treated to orient the liquid crystal molecules in order to introduce a twist of, e.g., 90°, between the substrates. Thus, the plane of polarization of plane polarized light will be rotated in a 90° angle as it passes through the twisted liquid crystal composition from one surface of the cell to the other surface. Application of an electric field between the selected electrodes of the cell causes the twist of the liquid crystal composition to be temporarily removed in the portion of the cell between the selected electrodes. By use of optical polarizers on each side of the cell, polarized light can be passed through the cell or extinguished, depending on whether or not an electric field is applied.

The polymeric alignment layer described above may be any of the materials commonly used in the liquid crystal art. Such materials include polyimides, polyvinyl alcohol, methyl cellulose, etc.

The transparent conducting layer described above is also conventional in the liquid crystal art. Such materi-

als include indium tin oxide, indium oxide, tin oxide, cadmium stannate, etc.

The dye image-receiving layer used in forming the color filter array element of the invention may comprise, for example, those polymers described in U.S. Pat. Nos. 4,695,286, 4,740,797, 4,775,657, and 4,962,081, the disclosures of which are hereby incorporated by reference. In a preferred embodiment, polycarbonates having a glass transition temperature greater than about 200° C. are employed. In another preferred embodiment, polycarbonates derived from a methylene substituted bisphenol-A are employed such as 4,4'-(hexahydro-4,7-methanoindan-5-ylidene)-bisphenol. In general, good results have been obtained at a coverage of from about 0.25 to about 5 mg/m<sup>2</sup>.

The support used in the invention is preferably glass such as borax glass, borosilicate glass, chromium glass, crown glass, flint glass, lime glass, potash glass, silica-flint glass, soda glass, and zinc-crown glass. In a preferred embodiment, borosilicate glass is employed.

Various methods may be used to transfer dye from the dye donor to the transparent support to form the color filter array element of the invention. There may be used, for example, a high intensity light flash technique with a dye-donor containing an energy absorptive material such as carbon black or a light-absorbing dye. Such a donor may be used in conjunction with a mirror which has a grid pattern formed by etching with a photoresist material. This method is described more fully in U.S. Pat. No. 4,923,860.

Another method of transferring dye from the dye donor to the transparent support to form the color filter array element of the invention is to use a heated embossed roller as described more fully in U.S. Pat. No. 4,978,652.

In another embodiment of the invention, the imagewise-heating is done by means of a laser using a dye-donor element comprising a support having thereon a dye layer and an absorbing material for the laser, the imagewise-heating being done in such a way as to produce a repeating mosaic pattern of colorants.

Any material that absorbs the laser energy or high intensity light flash described above may be used as the absorbing material such as carbon black or non-volatile infrared-absorbing dyes or pigments which are well known to those skilled in the art. In a preferred embodiment, cyanine infrared absorbing dyes are employed as described in U.S. Pat. No. 4,973,572, the disclosure of which is hereby incorporated by reference.

After the dyes are transferred to the receiver, the image may be treated to further diffuse the dye into the dye-receiving layer in order to stabilize the image. This may be done by radiant heating, solvent vapor, or by contact with heated rollers. The fusing step aids in preventing fading and surface abrasion of the image upon exposure to light and also tends to prevent crystallization of the dyes. Solvent vapor fusing may also be used instead of thermal fusing.

A process of forming a color filter array element according to the invention comprises

a) imagewise-heating a dye-donor element comprising a support having thereon a dye layer as described above, and

b) transferring portions of the dye layer to a dye-receiving element comprising a support having thereon a dye-receiving layer,

the imagewise-heating being done in such a way as to produce a repeating pattern of dyes to form the color filter array element.

A dye-donor element that is used to form the color filter array element of the invention comprises a support having thereon a mixture of dyes to form a green hue as described above along with other colorants such as imaging dyes or pigments to form the red and blue areas. Other imaging dyes can be used in such a layer provided they are transferable to the dye-receiving layer of the color array element of the invention by the action of heat. Especially good results have been obtained with sublimable dyes. Examples of additive sublimable dyes include anthraquinone dyes, e.g., Kayalon Polyol Brilliant Blue N BGM (R) Kayalon Polyol Brilliant Blue N-BGM (R) (Nippon Kayaku Co., Ltd.); azo dyes such as Kayalon Polyol Brilliant Blue BM (R) and Kayalon Polyol Dark Blue 2BM (R) (Nippon Kayaku Co., Ltd.); direct dyes such as Direct Dark Green B (R) (Mitsubishi Chemical Industries, Ltd.); basic dyes such as Sumiacryl Blue 6G (R) (Sumitomo Chemical Co., Ltd.), and Aizen Malachite Green (R) (product of Hodogaya Chemical Co., Ltd.). Examples of subtractive dyes useful in the invention include the following:



or any of the dyes disclosed in U.S. Pat. No. 4,541,830. 40  
The above cyan, magenta, and yellow subtractive dyes  
may be employed in various combinations, either in the  
dye-donor itself or by being sequentially transferred to  
the dye image-receiving element, to obtain the other  
desired blue and red additive primary colors. The dyes 45  
may be mixed within the dye layer or transferred se-  
quentially if coated in separate dye layers. The dyes  
may be used at a coverage of from about 0.05 to about  
1 g/m<sup>2</sup>.

The imaging dye, and an infrared-absorbing material 50 if one is present, are dispersed in the dye-donor element in a polymeric binder such as a cellulose derivative, e.g., cellulose acetate hydrogen phthalate, cellulose acetate, cellulose acetate propionate, cellulose acetate butyrate, cellulose triacetate; a polycarbonate; poly(styrene-co- 55 acrylonitrile), a poly(sulfone) or a poly(phenylene oxide). The binder may be used at a coverage of from about 0.1 to about 5 g/m<sup>2</sup>.

The dye layer of the dye-donor element may be coated on the support or printed thereon by a printing technique such as a gravure process. 60

Any material can be used as the support for the dye-donor element provided it is dimensionally stable and can withstand the heat generated by the thermal transfer device such as a laser beam. Such materials include 65 polyesters such as poly(ethylene terephthalate); polyamides; polycarbonates; glassine paper; condenser paper; cellulose esters; fluorine polymers; polyethers;

polyacetals; polyolefins; and polyimides. The support generally has a thickness of from about 2 to about 250  $\mu\text{m}$ . It may also be coated with a subbing layer, if desired.

5 Several different kinds of lasers could conceivably be used to effect the thermal transfer of dye from a donor sheet to the dye-receiving element to form the color filter array element in a preferred embodiment of the  
10 invention, such as ion gas lasers like argon and krypton; metal vapor lasers such as copper, gold, and cadmium; solid state lasers such as ruby or YAG; or diode lasers such as gallium arsenide emitting in the infrared region  
15 from 750 to 870 nm. However, in practice, the diode lasers offer substantial advantages in terms of their small size, low cost, stability, reliability, ruggedness, and ease of modulation. In practice, before any laser can be used to heat a dye-donor element, the laser radiation must be  
20 absorbed into the dye layer and converted to heat by a molecular process known as internal conversion. Thus, the construction of a useful dye layer will depend not only on the hue, sublimability and intensity of the image dye, but also on the ability of the dye layer to absorb the  
25 radiation and convert it to heat.

Lasers which can be used to transfer dye from the dye-donor element to the dye image-receiving element to form the color filter array element in a preferred embodiment of the invention are available commercially. There can be employed, for example, Laser Model SDL-2420-H2® from Spectrodiode Labs, or Laser Model SLD 304 V/W® from Sony Corp.

35 The following example is provided to illustrate the invention.

### EXAMPLE

40 A cyan dye-donor was prepared by coating on a  
 41 gelatin subbed transparent 175  $\mu\text{m}$  poly(ethylene tere-  
 42 phthalate) support a dye layer containing cyan dye 1  
 43 illustrated above ( $0.32 \text{ g/m}^2$ ) in a cellulose acetate prop-  
 44 ionate (2.5% acetyl, 46% propionyl) binder ( $0.27 \text{ g/m}^2$ )  
 45 coated from a 1-propanol, 2-butanone, toluene  
 and cyclopentanone solvent mixture. The dye layer also  
 46 contained Regal 300® (Cabot Co.) ( $0.22 \text{ g/m}^2$ ) ball-  
 47 milled to submicron particle size, Fluorad FC-431®  
 48 dispersing agent (3M Company) ( $0.01 \text{ g/m}^2$ ) and Solsp-  
 49 erse® 24000 dispersing agent (ICI Corp.) ( $0.03 \text{ g/m}^2$ )

Similar cyan dye-donors were prepared but using cyan dye 14 (0.15 g/m<sup>2</sup>) and cyan dye 15 (0.31 g/m<sup>2</sup>)

Control cyan dye-donors were prepared as described above but using Cyan Control Dye C-1 (0.48 g/m<sup>2</sup>), Cyan Control Dye C-2 (0.84 g/m<sup>2</sup>) and Cyan Control Dye C-3 (0.72 g/m<sup>2</sup>), as follows:





transferred as described to the same area of the receiver where the yellow dye was transferred to produce a green-hued image.

Each transferred test sample was placed in a sealed 5 chamber saturated with dichloromethane vapors for 5 minutes at 20° C. to diffuse the dyes into the receiver layer. The transferred dye images was then placed under a Pyropanel No. 4083 ® infrared heat panel at 210° C. for 60 sec. to remove residual solvent.

10 The Blue and Red Status A densities of the transferred dye image were read. The dye images were placed in an oven at 180° C. for two hours and the densities were re-read to determine percent dye loss due to heat fade. The following results were obtained:

TABLE

| Donor with<br>Cyan Dye | Donor with<br>Yellow Dye | STATUS A RED DENSITY |        |        | STATUS A BLUE DENSITY |        |        | Red Loss<br>minus<br>Blue Loss |
|------------------------|--------------------------|----------------------|--------|--------|-----------------------|--------|--------|--------------------------------|
|                        |                          | Initial              | Heated | % Loss | Initial               | Heated | % Loss |                                |
| C-1                    | A                        | 1.7                  | 0.6    | 65     | 1.9                   | 1.8    | 6      | 59                             |
| C-2                    | A                        | 2.4                  | 1.1    | 53     | 1.8                   | 1.3    | 27     | 26                             |
| C-3                    | A                        | 2.0                  | 1.4    | 30     | 2.0                   | 1.6    | 18     | 12                             |
| 1                      | A                        | 1.9                  | 1.7    | 10     | 1.9                   | 1.6    | 11     | 1                              |
| 14                     | A                        | 1.8                  | 1.8    | <5     | 1.7                   | 1.6    | <5     | 0                              |
| 15                     | A                        | 2.0                  | 1.9    | <5     | 1.9                   | 1.9    | <5     | 0                              |
| C-1                    | B                        | 1.6                  | 0.6    | 62     | 1.5                   | 1.5    | <5     | 57                             |
| 1                      | B                        | 1.9                  | 1.7    | 11     | 1.4                   | 1.1    | 20     | 9                              |
| 14                     | B                        | 1.9                  | 1.8    | 5      | 1.5                   | 1.3    | 14     | 9                              |
| 15                     | B                        | 2.0                  | 2.0    | <5     | 1.5                   | 1.5    | <5     | 0                              |
| C-1                    | L                        | 1.9                  | 0.6    | 69     | 2.1                   | 1.9    | 7      | 62                             |
| 14                     | L                        | 1.9                  | 1.8    | 7      | 2.3                   | 2.1    | 8      | 1                              |
| C-1                    | H                        | 2.0                  | 0.6    | 70     | 1.3                   | 1.3    | <5     | 65                             |
| 14                     | H                        | 1.8                  | 1.7    | 5      | 1.6                   | 1.5    | <5     | 1                              |

## Cyan Control Dye C-3

A yellow dye-donor was prepared as described above except that it contained yellow dye A as identified above (0.27 g/m<sup>2</sup>).

Similar yellow dye-donors were prepared but using 40 yellow dye B as identified above (0.17 g/m<sup>2</sup>), yellow dye L as identified above (0.60 g/m<sup>2</sup>) and yellow dye H as identified above (0.31 g/m<sup>2</sup>).

A dye-receiver was prepared by spin-coating the following layers on a 1.1 mm thick flat-surfaced borosilicate glass: 45

1) Subbing layer of duPont VM-651 Adhesion Promoter as a 1% solution in a methanol-water solvent mixture (0.5 μm thick layer equivalent to 0.54 g/m<sup>2</sup>), and

2) Receiver layer of a polycarbonate of 4,4'-(hexahydro-4,7-methanoindene-5-ylidene)bisphenol (2.5 g/m<sup>2</sup>), as described in U.S. Pat. No. 4,962,081, from methylene chloride solvent.

After coating, the receiver plate was heated in an 55 oven at 90° C. for one hour to remove residual solvent.

The yellow dye-donor was placed face down upon the dye-receiver. A Mecablitz ® Model 45 (Metz AG Company) electronic flash unit was used as a thermal energy source. It was placed 40 mm above the dye-donor using a 45-degree mirror box to concentrate the energy from the flash unit to a 25 × 50 mm area. The dye transfer area was masked to 12 × 42 mm. The flash unit was flashed once to produce a transferred Status A Blue transmission density of between 1.0 and 2.0. 60

After the yellow dye was transferred to the dye receiver, a cyan dye containing dye donor was place face down upon the same dye receiver. The cyan dye was

35 The above results indicate that the receiver containing the oxopyrroline cyan dyes according to the invention had better heat stability than those with the control cyan dyes as indicated by more constant red density. Blue density values were of course more dependent on the specific yellow dye chosen in combination with the cyan dye, but in general showed adequate to good heat stability and better "balance" of red to blue density change with the oxopyrroline cyan dyes of the invention. When hues, such as green, are formed of two or more dyes, it is important that dye fade be balanced for the components. Otherwise, severe hue shifts may be noticed.

50 The invention has been described in detail with particular reference to preferred embodiments thereof, but it will be understood that variations and modifications can be effected within the spirit and scope of the invention.

What is claimed is:

1. A thermally-transferred color filter array element comprising a support having thereon a polymeric dye image-receiving layer containing a thermally-transferred image comprising a repeating pattern of colorants, one of the colorants being a mixture of a yellow dye and a cyan dye to form a green hue, said cyan dye having the formula:



wherein:

R<sup>1</sup> represents hydrogen; a substituted or unsubstituted alkyl group having from 1 to about 8 carbon atoms; a cycloalkyl group having from about 5 to about 8 carbon atoms; or an alkenyl group having from about 2 to about 8 carbon atoms;

R<sup>2</sup> and R<sup>3</sup> each independently represents hydrogen; a substituted or unsubstituted alkyl group having from 1 to about 8 carbon atoms; or a cycloalkyl group having from about 5 to about 8 carbon atoms;

or R<sup>2</sup> and R<sup>3</sup> may be taken together to form a ring; or a 5- or 6-membered heterocyclic ring may be formed with R<sup>2</sup> or R<sup>3</sup>, the nitrogen to which R<sup>2</sup> or R<sup>3</sup> is attached, and J which is an alkyl group ortho to the carbon attached to the nitrogen atom; each J independently represents hydrogen; halogen; a substituted or unsubstituted alkyl or alkoxy group from 1 to about 6 carbon atoms; or two adjacent J's may represent the atoms necessary to form a 6-membered, fused, aromatic, carbocyclic ring; and n is from 1 to 4.

2. The element of claim 1 wherein said receiving layer comprises a polycarbonate binder having a glass transition temperature greater than about 200° C.

3. The element of claim 2 wherein said polycarbonate is derived from 4,4'-(hexahydro-4,7-methanoindene-5-ylidene)bisphenol.

4. The element of claim 1 wherein R<sup>1</sup> is CH<sub>2</sub>CH=CH<sub>2</sub>, R<sup>2</sup> and R<sup>3</sup> are each n-C<sub>4</sub>H<sub>9</sub> and J is hydrogen.

5. The element of claim 1 wherein a 6-membered heterocyclic ring is formed with R<sup>3</sup>, the nitrogen to which R<sup>3</sup> is attached, and J which is ortho to the carbon attached to the nitrogen atom; and R<sup>2</sup> is n-C<sub>4</sub>H<sub>9</sub> or C<sub>2</sub>H<sub>5</sub>.

6. The element of claim 1 wherein said pattern is a mosaic pattern of a set of red, green and blue additive primaries.

7. The element of claim 6 wherein said primary colors are separated from each other by an opaque area.

8. The element of claim 1 wherein said thermally-transferred image is obtained using laser induction.

9. The element of claim 1 wherein said thermally-transferred image is obtained using a high intensity light flash.

10. The element of claim 1 wherein said support is glass.

11. A process of forming a color filter array element comprising:

a) imagewise-heating a dye-donor element comprising a support having thereon a dye layer, and

b) transferring portions of said dye layer to a dye-receiving element comprising a support having thereon a dye-receiving layer,

said imagewise-heating being done in such a way as to produce a repeating pattern of colorants, one of the colorants being a mixture of a yellow dye and a cyan dye to form a green hue, said cyan dye having the formula

55



wherein:

10 R<sup>1</sup> represents hydrogen; a substituted or unsubstituted alkyl group having from 1 to about 8 carbon atoms; a cycloalkyl group having from about 5 to about 8 carbon atoms; or an alkenyl group having from about 2 to about 8 carbon atoms;

15 R<sup>2</sup> and R<sup>3</sup> each independently represents hydrogen; a substituted or unsubstituted alkyl group having from 1 to about 8 carbon atoms; or a cycloalkyl group having from about 5 to about 8 carbon atoms;

or R<sup>2</sup> and R<sup>3</sup> may be taken together to form a ring; or a 5- or 6-membered heterocyclic ring may be formed with R<sup>2</sup> or R<sup>3</sup>, the nitrogen to which R<sup>2</sup> or R<sup>3</sup> is attached, and J which is an alkyl group ortho to the carbon attached to the nitrogen atom;

each J independently represents hydrogen; halogen; a substituted or unsubstituted alkyl or alkoxy group from 1 to about 6 carbon atoms; or two adjacent J's may represent the atoms necessary to form a 6-membered, fused, aromatic, carbocyclic ring; and n is from 1 to 4.

12. The process of claim 11 wherein said receiving layer comprises a polycarbonate binder having a glass transition temperature greater than about 200° C.

13. The process of claim 11 wherein said polycarbonate is derived from 4,4'-(hexahydro-4,7-methanoindene-5-ylidene)bisphenol.

14. The process of claim 11 wherein R<sup>1</sup> is CH<sub>2</sub>CH=CH<sub>2</sub>, R<sup>2</sup> and R<sup>3</sup> are each n-C<sub>4</sub>H<sub>9</sub> and J is hydrogen.

15. The process of claim 11 wherein a 6-membered heterocyclic ring is formed with R<sup>3</sup>, the nitrogen to which R<sup>3</sup> is attached, and J which is ortho to the carbon attached to the nitrogen atom; and R<sup>2</sup> is n-C<sub>4</sub>H<sub>9</sub> or C<sub>2</sub>H<sub>5</sub>.

16. The process of claim 11 wherein said dye-donor element contains an additional light-absorbing material.

17. The process of claim 16 wherein a laser is used to supply energy in said imagewise-heating step.

18. The process of claim 16 wherein a high intensity light flash is used to supply energy in said imagewise-heating step.

19. The process of claim 11 which includes a further step of heating the transferred image to further diffuse the dye into said dye-receiving layer.

20. The process of claim 11 which includes a further step of subjecting the transferred image to solvent vapor to further diffuse the dye into said dye-receiving layer.

\* \* \* \* \*

60